

# United States Patent

[11] 3,619,278

[72] Inventor **Zennosuke Ogawa**  
Gumma-ken, Japan  
[21] Appl. No. **826,723**  
[22] Filed **May 21, 1969**  
[45] Patented **Nov. 9, 1971**  
[73] Assignee **Shinetsu Chemical Company**  
Tokyo, Japan  
[32] Priority **June 4, 1968**  
[33] **Japan**  
[31] **43/38200**

2,673,843 3/1954 Humphrey et al. .... 117/161 X  
2,755,194 7/1956 Volkmann et al. .... 117/161 UX  
3,240,731 3/1966 Nitzsche et al. .... 117/161 X  
3,294,725 12/1966 Findlay et al. .... 117/161 X

Primary Examiner—William D. Martin  
Assistant Examiner—Theodore G. Davis  
Attorney—Toren & McGeady

[54] **PROCESS FOR TREATING TEXTILE MATERIALS**  
10 Claims, No Drawings

[52] U.S. Cl. .... **117/139.5 A**,  
117/138.8 A, 117/139.4, 117/161 ZA  
[51] Int. Cl. .... **D06m15/66**  
[50] Field of Search. .... **117/139.5**,  
A, 139.5 CD, 161 ZA, 135.5, 138.8 A, 139.4,  
260/29.2 M, 46.5 G

[56] **References Cited**  
UNITED STATES PATENTS  
2,635,040 4/1953 Rasmussen ..... 38/144

**ABSTRACT:** When textile materials are treated with a silicone rubber emulsion containing, as its principal component, organopolysiloxane, prepared by emulsion polymerization of organosilane or organosiloxane, which is represented by a unit formula:



in which R is a monovalent hydrocarbon radical containing from 1 to 18 carbon atoms and n is a mean value of from 1.9 to 2.1, the relative viscosity of which silicone rubber emulsion in a toluene solution at 25°C. is at least 1.8, the textile materials are provided with excellent flexibility and springiness, and what is more, when the silicone rubber emulsion is applied to textile materials together with known resin-finishing agents heretofore employed for the purpose of improving the properties of the textile materials, it will serve to prevent the reduction of the strength of the textile materials which is one of the disadvantages of the known textile-material treating agents.

## PROCESS FOR TREATING TEXTILE MATERIALS

## SUMMARY OF THE INVENTION

This invention relates to a process of treating textile materials, especially for the purpose of providing them with flexibility and springiness.

Textile materials on the market are usually treated with resin so that they may be crease- and shrinkage-resistant, but such fabrics are apt to feel hard and have inferior physical properties due to their reduced strength. To overcome the difficulties, silicone oil or others are employed as a softener together with the treating agents, but a comparatively large amount of resin has to be employed under a severe condition when carrying out the permanent press which has become very popular these days. Therefore the use of the softener mentioned above often fails to maintain the desired strength and flexibility of the fabrics.

Consequently, to solve the problem, such methods as impregnating textile materials with dimethyl polysiloxane oil and a peroxide compound, such as benzene peroxide, and heating them, or treating the textile materials with solutions containing as their principal components methyl hydrogen polysiloxane, hydroxyl-group-terminated dimethyl polysiloxane and an organic tin compound, have been suggested. But the former treatment has a disadvantage in practicing in that the peroxide compound may explode when heated or subjected to impact, and when the latter method is resorted to, the treating solution has to be adjusted every time it is used, because it is unstable and cannot stand a longer storage.

The above-mentioned silicone oil provides cellulosic fabrics with comparatively good flexibility, but when the textile materials are of synthetic fibers such as polyester, polyamide or a mixture of polyester and cotton, no sufficient flexibility can be expected to be imparted by the silicone oil.

On the other hand, there has been proposed a method for treating textile materials with silicone rubber emulsion, which comprises polymerizing a cyclic organosiloxane in the presence of acid or alkali as catalyst, and then dispersing it with an emulsifier. Such silicone rubber emulsion, however, has disadvantages in respect of its stability.

The present invention relates to a method of treating textile materials which is free from the above disadvantages. The primary object of the invention is to provide a process for treating textile materials which gives them excellent flexibility and springiness in order to improve their touch, and another object is to provide a process of treating textile materials in which emulsions, easy to handle and having excellent stability, are employed to give the above-mentioned effect. Still another object is to provide a process, which, even when employed in combination with known processes comprising the treatment with resin substances, gives superior touch to the textile materials, besides improving their tear resistance.

Still further objects of the present invention shall be made clear by the detailed description of the process given below.

The present invention is characterized by treating textile materials with a silicone rubber emulsion containing, as its principal component, organopolysiloxane, prepared by emulsion-polymerization of organosilane or organosiloxane, which is represented by the unit formula:



(in which R is a monovalent hydrocarbon radical containing from one to 18 carbon atoms and n is a mean value of from 1.9 to 2.1) whose relative viscosity in a toluene solution (1 g./100 cc.) at 25° C. is at least 1.8.

To give a more detailed explanation, the silicone rubber emulsion prepared by emulsion-polymerization of organosilane or organosiloxane, is an emulsion consisting of corpuscles smaller than 1 micron, so that it can stand a long storage, and when textile materials are treated with this silicone rubber emulsion, better flexibility and springiness than

those provided by the heretofore employed treating agents are obtained, and especially when the emulsion is employed together with the known resin-finishing agents, not only the flexibility and springiness and other physical properties of textiles are improved but also entire or partial reduction of their strength is prevented, which is apt to be brought about by the resin-finishing agents.

The silicone rubber emulsion employed in the process of the invention is prepared by emulsion polymerization of organosilanes such as alkoxy silanes, or of cyclic or low-molecular straight-chained organosiloxanes. For example, it is prepared from octamethyl tetracyclosiloxane which is emulsified in an acid-type anionic emulsifier such as alkyl sulfonate or alkylsulfate, and is polymerized until the desired polymerization degree is obtained, and subsequently neutralized with alkali.

Organopolysiloxane contained in said emulsion, which is represented by the above-mentioned unit formula, must not be of too small polymerization degree. The relative viscosity,  $\eta_r$ , of the polysiloxane, when measured at 25° C. in a toluene solution (1 g. of polysiloxane/100 cc. of toluene), must be 1.8 or above. If it is below 1.8, the textile materials treated with the emulsion will not acquire the desired excellent flexibility and other physical properties. The organic radical (R) contained in said organopolysiloxane is a hydrocarbon radical containing from one to 18 carbon atoms as mentioned before, and it is exemplified by saturated or unsaturated hydrocarbon groups such as methyl, ethyl, vinyl and allyl, and aromatic hydrocarbon groups such as phenyl. On the other hand, when the ratio of said organic radical to silicon atoms given by  $R/Si = n$  is smaller than 1.9 the textile materials treated with the emulsion will become hard and possess no excellent flexibility, so that the value of n is defined to be between 1.9 and 2.1.

The process of the present invention, for the treatment of textile materials, is carried out very easily in the manner in which the known resin-finishing method is practiced. In the first place, the silicone rubber emulsion prepared by emulsion-polymerization of organosilane or organosiloxane is diluted with water until the solid content of the solution becomes 0.1-5 percent by weight, then a textile material is dipped in the aqueous solution thus prepared and squeezed on a mangle so that the solution content of the textile material may be 30-200 percent. The solution-impregnated textile material is then dried at 80°-100° C. and further heated for 30 seconds 5 minutes at 120°-180° C. If necessary, the treated textile material may be subjected to soaping, washing with hot and/or cold water, and then dried. Apart from the dipping method, roller coating can be employed in order to apply the silicone rubber emulsion to the textile. The ratio of the silicone rubber component applied to the textile is generally 0.1-10 percent by weight of the textile.

The compatibility of the silicone rubber emulsion with inorganic salts can be improved by the addition of nonionic, anionic or cationic emulsifier or high molecular materials, such as polyoxyethylene alkylphenol ether, polyoxyethylene alkyl ether, or block copolymer of polyoxyethylene and polyoxypropylene, and said silicone rubber emulsion can be employed in conjunction with resin-finishing agents such as methylol melamine, methylol urea or methylol melamine urea, the amount of the resin-finishing agent added to the emulsion being preferably less than 300 g./l. of the emulsion so as not to impair the purpose of the invention; in such a case, to the emulsion may be added 50 percent solution of a hardening agent selected from the group consisting of zinc nitrate, magnesium chloride and an organic amine salt, in an amount of 5-30 percent of the resin contained in the emulsion. On the other hand, in practicing the method of the invention, various finishing agents containing as a principal component, polyethylene, silicone oil, polyacrylic ester, polyvinyl alcohol, polyvinyl acetate or fluorine-containing resin may be used together with the silicone rubber emulsion.

The process of the invention may be applicable to every kind of textile made of natural, semisynthetic or synthetic

fibers, as well as to mixed or blended fabrics, giving an excellent effect.

The invention will now be described by several examples, in which the parts and percent are parts and percent by weight, and the value of the relative viscosity,  $\eta_r$ , is the viscosity measured at 25° C. of the toluene solution of polysiloxane prepared by dissolving 1 g. of polysiloxane in 100 cc. of toluene. The values of the physical properties of the textile materials given by the treatment of the present invention were obtained as follows:

1. Tear resistance:

5 test pieces, 63.5 mm.  $\times$  100 mm. in size, were cut lengthwise, and another 5 of the same size, breadthwise, from the textile material subjected to the process of the invention, and each test piece was placed on an Elmendorf Tester, with a 20.5 mm. cut made with a sharp knife in the center of the test piece at a right angle to its longer side, and the tear resistance values (g.), both lengthwise and breadthwise, represented by the average of 5 values given by the test piece before the remaining 43 mm. was torn, were adopted.

2. Crease-recovery rate:

5 test pieces, 15 mm.  $\times$  40 mm. in size, were cut lengthwise, another 5 of the same size, breadthwise, from the textile material subjected to the process of the invention, and each 25 was folded into two so that the longer side might be halved. It was then put between two flat boards, and was allowed to stand for 5 minutes with a load of 500 g. on it. After this, the opening angle of the test piece was measured with a Monsanto crease-recovery tester, and the crease-recovery rate was calculated by the following equation:

$$(\%) = \frac{a}{180} \times 100$$

3. Measurement with Handle-O-Meter:

A test piece of the size of 20 cm.  $\times$  20 cm. was subjected to a test in which a Handle-O-Meter was employed, and the resistance which the test piece showed was measured with an electric load cell. The measurement was made on the test piece lengthwise and breadthwise, both on the right side and on the wrong side, and the result was shown by the total of the values obtained.

4. Resilience-recovery rate:

A test piece was subjected to 50 percent elongation either lengthwise or breadthwise for 1 minute, and 5 seconds after its length ( $l_1$ ) was measured, and the resilience recovery rate was calculated by the following equation:

$$\frac{2l_0 - l_1}{l_0} \times 100$$

10

where  $l_0$  is the original length of the test piece.

5. Stability of the treating solution:

The treating solution was put in a vessel and was allowed to stand for 5 hours. The degree of the stability was judged by the following standard.

5th degree: No separation of oil is observed at all.

4th degree: Some spots or scums of oil are observed on the surface.

3rd degree: Spots or scums of oil are observed all over the surface.

2nd degree: A thick layer of oil or of scums is observed on the top of the emulsion.

1st degree: The emulsion is decomposed and completely separated.

### PREPARATION OF THE TREATING SOLUTIONS

Emulsions E-O, whose compositions are given in table 1-b were prepared by the method of emulsion-polymerization, while emulsions A-D were prepared for comparative purposes by adding an emulsifier, a diluent and water in the ratios given in table 1-a to various organopolysiloxanes, and to these emulsions

were added a 50 percent aqueous solution of dimethylol hydroxyethylene urea(resin-finishing agent), a 50 percent aqueous solution of zinc nitrate (hardening agent), and water, in the ratio given in table 2, obtaining the treating solutions Nos. 1-30.

The stability of each treating solution as tested is also given in table 2. The results proved that the organopolysiloxane-containing treating solutions employed in practicing the method of the invention are more stable than the others used for comparative purposes.

TABLE 1-a

| Organopolysiloxanes                                   |           |       |                                  |    | Water, parts                        | Other additives, parts | Diameter of corpuscle ( $\mu$ ) |
|-------------------------------------------------------|-----------|-------|----------------------------------|----|-------------------------------------|------------------------|---------------------------------|
| Member of the series                                  | Viscosity | Parts | Emulsifier, parts                |    |                                     |                        |                                 |
| A. Dimethyl silicone oil                              | 1.01      | 30    | Polyoxyethylene lauryl ether, 3. | 67 |                                     |                        | 1-5                             |
| B. do                                                 | 1.24      | 30    | do                               | 67 | Toluene, 10; perchloroethylene, 9.. |                        | 1-5                             |
| C. Hydroxy-terminated methylpolysiloxane.             | 1.28      | 27    | Polyoxyethylene lauryl ether, 1. | 47 | do                                  |                        | 1-5                             |
| D. Methyl hydrogen polysiloxane.                      | 1.00      | 3     |                                  |    |                                     |                        | 1-5                             |
| Silicone rubber having a unit formula $(CH_3)_2SiO$ . | 2.14      | 15    | Polyoxyethylene cetyl ether, 5.  | 35 | Toluene, 20; perchloroethylene, 9.. |                        | 10-50                           |

TABLE 1-b

|                                                                                  |      |    |                                        |    |  |  |         |
|----------------------------------------------------------------------------------|------|----|----------------------------------------|----|--|--|---------|
| E. Silicone rubber having a unit formula $(CH_3)_2SiO$ .                         | 1.53 | 30 | Polyoxyethylene oleyl ether, 3.        | 67 |  |  | 0.1-0.5 |
| F. do                                                                            | 1.62 | 30 | do                                     | 67 |  |  | 0.1-0.5 |
| G. do                                                                            | 1.73 | 30 | do                                     | 67 |  |  | 0.1-0.5 |
| H. Silicone rubber having a unit formula $(CH_3)_{1.7}SiO_{1.5}$ .               | 1.96 | 30 | do                                     | 67 |  |  | 0.5-1.0 |
| I. Silicone rubber having a unit formula $(CH_3)_{1.8}SiO_{1.5}$ .               | (1)  | 30 | do                                     | 67 |  |  | 0.5-1.0 |
| J. Silicone rubber having a unit formula $(CH_3)_{1.9}SiO_{1.5}$ .               | 1.81 | 30 | do                                     | 67 |  |  | 0.1-0.5 |
| K. do                                                                            | 2.03 | 30 | do                                     | 67 |  |  | 0.1-0.5 |
| L. Silicone rubber having a unit formula $(CH_3)_{1.9}SiO_{1.5}$ .               | 1.96 | 30 | do                                     | 67 |  |  | 0.5-0.7 |
| M. Silicone rubber having a unit formula $(CH_3)_{1.9}(CH_2=CH)_0.1 SiO$ .       | 1.94 | 30 | Polyoxyethylene lauryl ether, 5.       | 65 |  |  | 0.3-0.5 |
| N. Silicone rubber having a unit formula $(CH_3)_{1.8}(C_6H_5)_0.03 SiO_{1.5}$ . | 1.87 | 50 | Polyoxyethylene nonyl phenyl ether, 3. | 47 |  |  | 1       |
| O. Silicone rubber having a unit formula $(CH_3)_{1.9}(C_{10}H_{20})_0.1 SiO$ .  | 1.98 | 30 | Polyoxyethylene cetyl ether, 5.        | 65 |  |  | 0.8-1   |

<sup>1</sup> Insoluble in toluene.

TABLE 2

| Treating solution number | Emulsion | Kind  | Parts | 50% aqueous solution of         | 50% aqueous solution of | Water, parts | Stability, degree |
|--------------------------|----------|-------|-------|---------------------------------|-------------------------|--------------|-------------------|
|                          |          |       |       | dimethylol ethylene urea, parts | zinc nitrate, parts     |              |                   |
| Control.....             | 1        | ..... | 0     | 7                               | 1                       | 92           | 5                 |
| Do.....                  | 2        | A     | 2     | 7                               | 1                       | 90           | 4                 |
| Do.....                  | 3        | B     | 2     | 7                               | 1                       | 90           | 3                 |
| Do.....                  | 4        | C     | 2     | 7                               | 1                       | 90           | 2                 |
| Do.....                  | 5        | D     | 4     | 7                               | 1                       | 88           | 1                 |
| Do.....                  | 6        | E     | 2     | 7                               | 1                       | 90           | 5                 |
| Do.....                  | 7        | F     | 2     | 7                               | 1                       | 90           | 5                 |
| Do.....                  | 8        | G     | 2     | 7                               | 1                       | 90           | 5                 |
| Do.....                  | 9        | H     | 2     | 7                               | 1                       | 90           | 5                 |
| Do.....                  | 10       | I     | 2     | 7                               | 1                       | 90           | 5                 |
| Example.....             | 11       | J     | 2     | 7                               | 1                       | 90           | 5                 |
| Do.....                  | 12       | K     | 2     | 7                               | 1                       | 90           | 5                 |
| Do.....                  | 13       | L     | 2     | 7                               | 1                       | 90           | 5                 |
| Do.....                  | 14       | M     | 2     | 7                               | 1                       | 90           | 5                 |
| Do.....                  | 15       | N     | 3     | 7                               | 1                       | 89           | 5                 |
| Do.....                  | 16       | O     | 3     | 7                               | 1                       | 89           | 5                 |
| Control.....             | 17       | ..... | 0     | 6                               | 1                       | 93           | 5                 |
| Do.....                  | 18       | A     | 1     | 6                               | 1                       | 92           | 4                 |
| Do.....                  | 19       | A     | 2     | 6                               | 1                       | 91           | 4                 |
| Example.....             | 20       | A     | 3     | 6                               | 1                       | 90           | 4                 |
| Do.....                  | 21       | J     | 1     | 6                               | 1                       | 92           | 5                 |
| Do.....                  | 22       | J     | 2     | 6                               | 1                       | 91           | 5                 |
| Do.....                  | 23       | J     | 3     | 6                               | 1                       | 90           | 5                 |
| Control.....             | 24       | ..... | 0     | 15                              | 2.3                     | 82.7         | 5                 |
| Do.....                  | 25       | A     | 1     | 15                              | 2.3                     | 81.7         | 3-4               |
| Do.....                  | 26       | A     | 2     | 15                              | 2.3                     | 80.7         | 3-4               |
| Example.....             | 27       | A     | 3     | 15                              | 2.3                     | 79.7         | 3-4               |
| Do.....                  | 28       | J     | 1     | 15                              | 2.3                     | 81.7         | 5                 |
| Do.....                  | 29       | J     | 2     | 15                              | 2.3                     | 80.7         | 5                 |
| Do.....                  | 30       | J     | 3     | 15                              | 2.3                     | 79.7         | 5                 |

TABLE 3

| Treating solution Number | Tear resistance, length-wise+breadth-wise, g. | Crease-recovery rate, percent | Value obtained by means of Handle-O-Meter (Slit: 10 mm.), g. |       | Touch                   |
|--------------------------|-----------------------------------------------|-------------------------------|--------------------------------------------------------------|-------|-------------------------|
|                          |                                               |                               | Handle-O-Meter                                               | Touch |                         |
| Control.....             | (1)                                           | 600                           | 51.1                                                         | 84.0  |                         |
| Do.....                  | 1                                             | 483                           | 64.0                                                         | 64.0  | Hard.                   |
| Do.....                  | 2                                             | 609                           | 66.2                                                         | 60.0  | Harsh.                  |
| Do.....                  | 3                                             | 733                           | 66.4                                                         | 58.0  | Slippery soft, limp.    |
| Do.....                  | 4                                             | 710                           | 67.3                                                         | 60.0  | Do.                     |
| Do.....                  | 5                                             | 781                           | 73.5                                                         | 59.0  | Slippery soft, springy. |
| Do.....                  | 6                                             | 695                           | 65.8                                                         | 59.5  | Slippery soft, limp.    |
| Do.....                  | 7                                             | 760                           | 67.1                                                         | 57.5  | Do.                     |
| Do.....                  | 8                                             | 762                           | 67.4                                                         | 59.5  | Do.                     |
| Do.....                  | 9                                             | 645                           | 69.7                                                         | 69.0  | Hard, stiff.            |
| Do.....                  | 10                                            | 596                           | 68.6                                                         | 72.3  | Do.                     |
| Example.....             | 11                                            | 780                           | 73.0                                                         | 58.5  | Slippery soft, springy. |
| Do.....                  | 12                                            | 770                           | 73.2                                                         | 58.7  | Do.                     |
| Do.....                  | 13                                            | 765                           | 73.8                                                         | 60.1  | Slightly hard; springy. |
| Do.....                  | 14                                            | 705                           | 88.1                                                         | 62.2  | Extremely springy.      |
| Do.....                  | 15                                            | 685                           | 68.9                                                         | 61.0  | Harsh, springy.         |
| Do.....                  | 16                                            | 845                           | 59.1                                                         | 57.8  | Slippery soft.          |

<sup>1</sup> Untreated cloth.

\* 0.5 part of an emulsion prepared by emulsifying 10 parts of dibutyl tin dioctoate, 10 parts of toluene, 1 part of polyoxoethylene lauryl alcohol, and 79 parts of water was added, as a hardening catalyst for organosiloxane, to the treating solution.

## EXAMPLE 1

Test pieces of cotton poplin (4OS') were each dipped into the treating solutions Nos. 1-16, mangled to the state containing 60 percent of the solution in relation to the weight of the cloth (weight of silicone component/weight of cloth: 0.36 percent), subjected to the preliminary heating at 100° C. for 3 minutes, then to the heat treatment at 160° C. for 3 minutes, followed by soaping, hot-water washing, cold-water washing and drying. The tear resistance, the crease-recovery rate, the value obtained by means of the Handle-O-Meter, and the touch of the test pieces thus treated are given in table 3.

## EXAMPLE 2

Just as in example 1, test pieces of cotton poplin (4OS') were treated with treating solutions Nos. 17-23, and the tear resistance, the crease-recovery rate, the value obtained by means of the Handle-O-Meter and the touch of the test pieces thus treated proved to be as given in table 4. It is clear from the table that the test pieces treated with emulsion J of the invention gave better softness, springiness and recovery of

crease than those treated with hitherto employed emulsion A consisting of silicone oil.

## EXAMPLE 3

Just as in example 1, test pieces of broadcloth (8OS' blend spun yarn) of 65 percent polyester fiber and 35 percent cotton were treated with treating solutions Nos. 24-30; and the tear resistance, the crease-recovery rate, the value obtained by means of Handle-O-Meter and the touch of the test pieces thus treated proved to be as given in table 5. It was found, as in example 2, that the treating solution, emulsion J, of the invention served to improve the physical properties of the textile materials better than emulsion A consisting of silicone oil.

## EXAMPLE 4

4 parts of emulsion A and emulsion J were each diluted with 96 parts of water, obtaining treating solution Nos. 31 and 32. Test pieces of tricot (100 percent polyester fiber) were dipped into either of the treating solutions, mangled and dried at 100° C. for 4 minutes. The test pieces thus treated proved to have 1.2 percent by weight of silicone per 100 percent by weight of the textile material. The values obtained the Handle-O-Meter and the resilience recovery rates of the test pieces were as given in table 6.

TABLE 4

| Treating solution number | Tear resistance, lengthwise+breadthwise, g. | Crease-recovery rate, percent | Value obtained by means of Handle-O-Meter (slit: 10 mm.), g. | Touch                   |
|--------------------------|---------------------------------------------|-------------------------------|--------------------------------------------------------------|-------------------------|
| Control.....             | 620                                         | 51.1                          | 82.2                                                         |                         |
| Do.....                  | 515                                         | 64.0                          | 64.0                                                         | Hard.                   |
| Do.....                  | 640                                         | 64.7                          | 62.0                                                         |                         |
| Do.....                  | 663                                         | 66.8                          | 61.5                                                         | Harsh.                  |
| Do.....                  | 671                                         | 68.0                          | 60.0                                                         |                         |
| Example.....             | 680                                         | 73.9                          | 58.5                                                         |                         |
| Do.....                  | 712                                         | 75.0                          | 58.0                                                         | Slippery soft, springy. |
| Do.....                  | 757                                         | 75.1                          | 56.0                                                         |                         |

TABLE 5

| Treating solution number | Tear resistance, lengthwise+breadthwise, g. | Crease-recovery rate, percent | Value obtained by means of Handle-O-Meter (slit: 10 mm.), g. | Touch                    |
|--------------------------|---------------------------------------------|-------------------------------|--------------------------------------------------------------|--------------------------|
| Control.....             | 1,201                                       | 67.3                          | 137                                                          |                          |
| Do.....                  | 1,184                                       | 83.3                          | 121                                                          | Hard.                    |
| Do.....                  | 1,233                                       | 83.4                          | 122                                                          |                          |
| Do.....                  | 1,283                                       | 83.5                          | 122                                                          | Lacking in flexibility,  |
| Do.....                  | 1,367                                       | 84.7                          | 120                                                          | rather hard in the core. |
| Example.....             | 1,650                                       | 84.8                          | 109                                                          |                          |
| Do.....                  | 1,661                                       | 86.9                          | 109                                                          |                          |
| Do.....                  | 1,683                                       | 87.5                          | 107                                                          | Slippery soft, springy.  |

TABLE 6

| Treating solution Number | Value obtained by means of Handle-O-Meter (Slit: 15 mm.), g. | Resilience recovery rate, percent |              |                                             | Remarks |
|--------------------------|--------------------------------------------------------------|-----------------------------------|--------------|---------------------------------------------|---------|
|                          |                                                              | Length-wise                       | Breadth-wise |                                             |         |
| Untreated cloth.         | 282.0                                                        | 91                                | 90           | Control.                                    |         |
| 31.....                  | 281.5                                                        | 92                                | 93           | Do.                                         |         |
| 32.....                  | 261.5                                                        | 95                                | 95           | Treating solution of the present invention. |         |

TABLE 7

| Treating solution Number | Value obtained by means of Handle-O-Meter (Slit: 15 mm.), g. | Resilience recovery rate, percent |              |                                             | Remarks |
|--------------------------|--------------------------------------------------------------|-----------------------------------|--------------|---------------------------------------------|---------|
|                          |                                                              | Length-wise                       | Breadth-wise |                                             |         |
| Untreated cloth.         | 205                                                          | 90                                | 83           | Control.                                    |         |
| 33.....                  | 196                                                          | 94                                | 93           | Do.                                         |         |
| 34.....                  | 148                                                          | 98                                | 97           | Treating solution of the present invention. |         |

TABLE 8

| Treating solution Number | Value obtained by means of Handle-O-Meter (Slit: 15 mm.), g. | Resilience recovery rate, percent |              |                                             | Remarks |
|--------------------------|--------------------------------------------------------------|-----------------------------------|--------------|---------------------------------------------|---------|
|                          |                                                              | Length-wise                       | Breadth-wise |                                             |         |
| Untreated cloth.         | 195                                                          | 90                                | 90           | Control.                                    |         |
| 35.....                  | 186                                                          | 90                                | 91           | Do.                                         |         |
| 36.....                  | 143                                                          | 95                                | 95           | Treating solution of the present invention. |         |

The test pieces treated with treating solution No. 32 proved to possess excellent touch, being very pliable and flexible.

#### EXAMPLE 5

10 parts of emulsion A and emulsion J were each diluted with 90 parts of water, obtaining treating solution Nos. 33 and 34. Test pieces of jersey of 100 percent polyamide resin fiber were dipped into either of them, mangled and dried at 100°C. for 5 minutes. The test pieces thus treated proved to have 3.1 percent by weight of silicone per 100 percent by weight of the textile material. Tests described in example 4 were conducted on them, giving the results shown in table 7.

The test pieces treated with treating solution No. 34 proved to possess excellent touch, being very pliable and elastic.

#### EXAMPLE 6

5 parts of emulsion A and emulsion F were each diluted with 95 parts of water, obtaining treating solution Nos. 31 and

32. Test pieces of jersey of 100 percent acrylonitrile fiber were dipped into either of them, mangled, and dried at 100°C. for 5 minutes. The test pieces thus treated proved to have 1.8 percent by weight of silicone per 100 percent by weight of the textile material. Tests described in example 4 were conducted on them, giving the results shown in table 8.

30 The test pieces treated with treating solution No. 36 proved to possess excellent touch, being very pliable, flexible and slippery soft.

We claim:

1. A process of treating textile materials which is characterized by treating them with a silicone rubber emulsion, containing, as its principal component, organopolysiloxane, prepared by emulsion polymerization of organosilicone compounds selected from organosilane and organosiloxane, which is represented by a unit formula;



45 where R is a monovalent hydrocarbon radical containing from one to 18 carbon atoms and n is a mean value of from 1.9 to 2.1, whose relative viscosity in a toluene solution at 25°C. is at least 1.8, applying to said textiles said organopolysiloxane at the ratio of 0.1 to 10 percent by weight of the textile materials, and then drying at 80° to 100°C.

50 2. The process of claim 1 which is characterized by treating textile materials with the said silicone rubber emulsion, containing organopolysiloxane in the amount ranging between 0.1 and 5 percent by weight of the silicone rubber emulsion.

55 3. The process of claim 1 which is characterized by treating textile materials with the said silicone rubber emulsion to which has been mixed an emulsifier, where R is a monovalent hydrocarbon radical containing from 1 to 18 carbon atoms and n is a mean value of from 1.9 to 2.1, whose relative viscosity in a toluene solution at 25°

60 4. The process of claim 1 which is characterized by treating textile materials with the said silicone rubber emulsion to which has been added a resin-finishing agent, selected from the group consisting of methylol melamine methylol urea, methylol melamine urea and dimethylol dihydroxyethylene urea, in the amount of less than 300 g./l. of said emulsion, in the presence of a 50 weight percent solution of a hardening agent selected from the group consisting of zinc nitrate, magnesium chloride and organic amine salt, in an amount of 5-30 percent by weight of the resin contained in the emulsion.

5. The process of claim 4 which is characterized by treating textile materials with said silicone rubber emulsion to which has been added said resin finishing agent, selected from the group consisting of methylol melamine urea, methylol melamine urea and dimethylol dihydroxyethylene urea, in the amount of less than 300 g./l. of said emulsion, in the presence of a 50 weight percent solution of a hardening agent selected from the group consisting of zinc nitrate, magnesium chloride and organic amine salt, in an amount of 5-30 percent by weight of the resin contained in the emulsion.

6. A process of treating textile materials which is characterized by dipping them in a silicone rubber emulsion, containing as its principal component, organopolysiloxane, prepared by emulsion-polymerization of organosilicone compounds selected from organosilane and organosiloxane, which is represented by a unit formula:



where R is a monovalent hydrocarbon radical, containing from 1 to 18 carbon atoms and n is a mean value of from 1.9 to 2.1, whose relative viscosity in a toluene solution at 25° C. is at least 1.8, then mangling them to the state of containing from 30 to 200 percent of the solution in relation to the weight of the textile materials, drying them at 80°-100° C. and further heating them for 30 seconds—5 minutes at 120°-180° C.

7. The process of claim 6 which is characterized by treating textile materials with said silicone rubber emulsion, containing organopolysiloxane in the amount ranging between 0.1 and 5 percent by weight of the silicone rubber emulsion.

8. The process of claim 6 which is characterized by treating textile materials with said silicone rubber emulsion to which has been added a resin-finishing agent, selected from the group consisting of methylol melamine, methylol urea, methylol melamine urea and dimethylol dihydroxyethylene urea, in the amount of less than 300 g./l. of said emulsion.

9. The process of claim 6 which is characterized by treating textile materials with said silicone rubber emulsion to which has been added a resin-finishing agent, selected from the

10 group consisting of methylol melamine, methylol urea, methylol melamine urea and dimethylol dihydroxyethylene urea, in the amount of less than 300 g./l. of said emulsion, in the presence of 50 weight percent solution of a hardening agent, selected from the group consisting of zinc nitrate, magnesium chloride and organic amine salt, in an amount of 5 to 30 percent by weight of the resin contained in the emulsion.

15 10. The process of claim 6 which is characterized by treating textile materials with said silicone rubber emulsion to which has been mixed an emulsifier.

\* \* \* \* \*